# EUROPEAN PATENT SPECIFICATION

(11) **EP 1 052 110 B1**
(45) Date of publication and mention of the grant of the patent: **12.05.2004**
(21) Application number: 99303789.4
(22) Date of filing: 14.05.1999
(51) Int. Cl.: B41M 5/00

(54) **Transparent plastic writing sheet**
Durchsichtige Aufzeichnungskunststofffolie
Feuille en plastique transparente pour l'écriture

(43) Date of publication of application: 15.11.2000
(73) Proprietor: Taiwan Hopax Chemicals Mfg., Co., Ltd, Feng-Shang City, Kaohsiung Hsien (TW)
(72) Inventor: Lin, Bin-Tzer, Taipei City (TW); Kuo, Tsung-Tien, Niao-Sung Hsiang, Kaohsiung Hsien (TW); Hsieh, Hsieh-Chang, Feng-Shan City, Kaohsiung Hsien (TW); Liu, Jen-Rong, Feng-Shan City, Kaohsiung Hsien (TW); Lin, Ho-Tsai, Nan-Tzu Dist., Kaohsiung City (TW)
(74) Representative: Ritter, Stephen David

(56) References cited:
- EP-A- 0 365 712
- EP-A- 0 444 950
- EP-A- 0 696 516
- WO-A-96/31353
- US-A- 5 888 635

## Description

This invention relates to a writing sheet, more particularly to a transparent writing sheet coated with a layer of transparent coating that possesses excellent writing quality.

Self-stick writing sheets have become popular in recent years since they can be attached on a surface of a table, a wall, a book or a document as desired. However, conventional self-stick writing sheets are normally made of paper, thereby suffering from the following drawbacks that (1) they are prone to break upon use due to the lack of tensile strength for paper, and (2) they are not waterproof.

It is known that polypropylene can be used to fabricate synthetic paper with writing quality, printability, waterproof, and good tensile strength. However, since the writing quality of the synthetic paper is still poor in comparison with common papers, such as poor ink absorbability, there remains a need for improving the writing quality for the synthetic paper. In addition, synthetic paper is not transparent.

Therefore, it is an object of the present invention to provide a writing sheet that has good tensile strength and excellent writing quality, and that is water-proof and transparent.

EP-A-0 696 516 and US 5,888,635 disclose an ink jet recording medium which comprises: (i) a base substrate which can be a transparent, translucent or opaque plastic or a paper, (ii) an underlayer on one surface of the base substrate, wherein the underlayer comprises one or more polymeric materials, in which at least one polymeric material is a water-imbibing component, and (iii) a surface layer disposed of on a surface of the underlayer, wherein the surface layer comprises one or more inorganic particulates.

According to the present invention, a writing sheet comprises a transparent plastic film directly coated with a layer of transparent coating, the coating layer being prepared from a mixture of a binder and at least one pigment, the binder being selected from the group consisting of polyvinyl alcohol, polyacrylate, polyvinyl acetate, and styrene butadiene rubber, the pigment being selected from the group consisting of titanium dioxide, calcium carbonate, clay, and mixtures thereof. The weight ratio of the binder to the pigment ranges from 1:1 to 1:10.

In drawings which illustrate the preferred embodiment of the invention,
Fig. 1 illustrates a side view of a self-stick writing sheet of a preferred embodiment of this invention; and
Fig. 2 illustrates a plurality of the self-stick writing sheets of Fig. 1 arranged in a stack.

Fig. 1 illustrates a side view of a writing sheet embodying this invention. The writing sheet 1 of the present invention includes a plastic film 11 coated with a layer of removable adhesive 111 on the bottom side of the writing sheet 1 and a layer of transparent coating 112 on the top side of the writing sheet 1. The coating 112 provides a mat writing face. A plurality of the writing sheets 1 are assembled to form a stack of self-stick notes 2 (see Fig. 2) by stacking the writing sheets 1 one above the other with the bottom side of each writing sheet 1 in contact with the top side of an adjacent sheet 1.

The plastic film 11 is made from a material selected from the group consisting of polypropylene, polyethylene, polyvinyl chloride, polyethylene terephthalate, and Mylar^{RTM}.

The removable adhesive 111 may be any one of pressure sensitive adhesives known in the art. A typical example of the removable adhesive 111 is an acrylate-type adhesive.

The coating 112 of the writing sheet 1 comprises a mixture of a binder and at least one pigment. The binder of the coating 112 is preferably selected from the group consisting of polyvinyl alcohol, polyacrylate, polyvinyl acetate, and styrene butadiene rubber. The pigment of the coating 112 is preferably selected from the group consisting of titanium dioxide, calcium carbonate, clay, and mixtures thereof. The weight ratio of the binder to the pigment preferably ranges from 1:1 to 1:10 so as to render the coating of the writing sheet 1 of this invention to possess a transparent characteristic with excellent writing quality.

The coating of the writing sheet 1 can further include a dye so as to color the writing sheet 1. The dye may be added in an amount of more than 2% by weight based on the total weight of the pigment.

The writing sheet 1 of this invention can further include a release paper (not shown) for covering and protecting the coating layer 112 of the plastic film 11.

### EXAMPLES

Tests were done for investigating the writing quality of samples of the writing sheet of this invention. The writing quality of the writing sheet is classified into three rankings which are represented as excellent (e), good (g) , and fair (f) , and is determined based on the writability, anchorage ( a binding power of the pigment to the film ) , and ink absorbability.

Polypropylene was used as a plastic film in each of the samples. The coatings on the samples were prepared from different combinations of binders and pigments with differing weight ratios of binder to pigment. The binders used in these tests were polyvinyl alcohol (PVA), polyvinyl acetate (PA), and styrene butadiene rubber (SBR). The pigments used in these tests were titanium dioxide(TiO₂), calcium carbonate (CaCO₃), and clay. The weight ratios of the binder to the pigment arranged in these tests ranged from 1 : 10 to 1 : 1 which are expressed in terms of grams of binder per 100 g of pigment in Tables 1-3.

**Table 1**

| Sample # | TiO₂ g | Clay g | CaCO₃ g | PVA g | Sample # | TiO₂ g | Clay g | CaCO₃ g | PVA g |
|---|---|---|---|---|---|---|---|---|---|
| 1 | 100 | - | - | 100 | 11 | - | 100 | - | 25 |
| 2 | 100 | - | - | 75 | 12 | - | 100 | - | 20 |
| 3 | 100 | - | - | 50 | 13 | - | 100 | - | 15 |
| 4 | 100 | - | - | 25 | 14 | - | 100 | - | 10 |
| 5 | 100 | - | - | 20 | 15 | - | 100 | - | 5 |
| 6 | 100 | - | - | 15 | 16 | - | - | 100 | 75 |
| 7 | - | 100 | - | 100 | 17 | - | - | 100 | 50 |
| 8 | - | 100 | - | 75 | 18 | - | - | 100 | 30 |
| 9 | - | 100 | - | 50 | 19 | - | - | 100 | 20 |
| 10 | - | 100 | - | 30 | - | - | - | - | - |

**Table 2**

| Sample # | TiO₂ g | Clay g | CaCO₃ g | PA g | Sample # | TiO₂ g | Clay g | CaCO₃ g | PA g |
|---|---|---|---|---|---|---|---|---|---|
| 20 | - | - | 100 | 100 | 28 | 100 | - | - | 25 |
| 21 | - | - | 100 | 75 | 29 | 100 | - | - | 5 |
| 22 | - | - | 100 | 50 | 30 | - | 100 | - | 100 |
| 23 | - | - | 100 | 25 | 31 | - | 100 | - | 75 |
| 24 | - | - | 100 | 5 | 32 | - | 100 | - | 50 |
| 25 | 100 | - | - | 100 | 33 | - | 100 | - | 25 |
| 26 | 100 | - | - | 75 | 34 | - | 100 | - | 5 |
| 27 | 100 | - | - | 50 | - | - | - | - | - |

**Table 3**

| Sample # | TiO₂ g | Clay g | CaCO₃ g | SBR g | Sample # | TiO₂ g | Clay g | CaCO₃ g | SBR g |
|---|---|---|---|---|---|---|---|---|---|
| 35 | 100 | - | - | 100 | 42 | - | 100 | - | 25 |
| 36 | 100 | - | - | 75 | 43 | - | 100 | - | 5 |
| 37 | 100 | - | - | 50 | 44 | - | - | 100 | 100 |
| 38 | 100 | - | - | 25 | 45 | - | - | 100 | 75 |
| 39 | - | 100 | - | 100 | 46 | - | - | 100 | 50 |
| 40 | - | 100 | - | 75 | 47 | - | - | 100 | 25 |
| 41 | - | 100 | - | 50 | 48 | - | - | 100 | 5 |

Samples #1-#19 are listed in Table 1, samples #20-#34 in Table 2, and samples #35-#48 in Table 3.

The results of these tests were shown in Table 4. To summarize from the results shown in Table 4, samples #1-#2 which contain TiO₂, samples #12-#14, #33-#34 and #42-#43 which contain clay, and samples #19, and #45-#47 which contain CaCO₃ exhibit good and/or excellent writability, anchorage, and as well as ink absorbability.

**Table 4**

| Sample # | Writability | Anchorage | Ink absorbability | Sample # | Writability | Anchorage | Ink absorbability |
|---|---|---|---|---|---|---|---|
| 1 | e | g | e | 25 | f | e | f |
| 2 | e | g | e | 26 | f | e | f |
| 3 | e | f | g | 27 | f | g | e |
| 4 | g | f | g | 28 | g | g | g |
| 5 | g | g | g | 29 | peeling | - | - |
| 6 | f | f | e | 30 | f | g | f |
| 7 | f | f | e | 31 | f | e | f |
| 8 | f | f | e | 32 | f | e | f |
| 9 | e | f | f | 33 | g | e | g |
| 10 | f | f | e | 34 | e | e | g |
| 11 | g | f | e | 35 | g | e | f |
| 12 | g | g | g | 36 | e | e | f |
| 13 | g | g | g | 37 | e | e | f |
| 14 | g | e | g | 38 | g | f | f |
| 15 | g | e | f | 39 | g | e | f |
| 16 | e | f | g | 40 | g | e | f |
| 17 | e | f | f | 41 | g | e | f |
| 18 | e | f | F | 42 | e | e | g |
| 19 | e | g | g | 43 | g | g | g |
| 20 | f | e | f | 44 | g | e | f |
| 21 | f | g | f | 45 | e | e | g |
| 22 | e | g | f | 46 | g | e | g |
| 23 | g | g | f | 47 | g | g | g |
| 24 | g | g | f | 48 | g | f | g |

It will be appreciated that the specific examples of writing sheets referred to herein include adhesive labels. Such adhesive labels encompass labels which may be permanently affixed to a substrate and labels which are readily removable or repositionable (c.f. Post-it^{RTM} notes).

## Claims

1. A writing sheet **characterized by** a transparent plastic film (11) directly coated with a layer of transparent coating (112), said coating layer (112) being prepared from a mixture of a binder and at least one pigment, said binder being selected from the group consisting of polyvinyl alcohol, polyacrylate, polyvinyl acetate, and styrene butadiene rubber, said pigment being selected from the group consisting of titanium dioxide, calcium carbonate, clay, and mixtures thereof, the weight ratio of said binder to said pigment ranges from 1:1 to 1:10.

2. The writing sheet of Claim 1, **characterized in that** said plastic film (11) is made from a material selected from the group consisting of polypropylene, polyethylene, polyvinyl chloride and polyethylene terephthalate.

3. The writing sheet of Claim 1 or Claim 2, further **characterized by** a layer of removable adhesive (111) applied to said plastic film (11) to provide said writing sheet (1) with a removable sticking characteristic.

4. The writing sheet of any of Claims 1 to 3, further **characterized by** a release paper that covers said coating layer (112) of said plastic film (11).

5. The writing sheet of Claim 1, **characterized in that** said binder is polyvinyl alcohol, and said pigment is titanium dioxide, wherein the weight ratio of polyvinyl alcohol to titanium dioxide is from 1:1 to 1:2.

6. The writing sheet of Claim 1, **characterized in that** said binder is styrene butadiene rubber, and said pigment is calcium carbonate, wherein the weight ratio of styrene butadiene rubber to calcium carbonate is from 1:1 to 1:2.

7. The writing sheet of Claim 1, **characterized in that** said coating further includes a dye.

## Patentansprüche

1. Schreibbogen, **gekennzeichnet durch** einen transparenten Kunststofffilm (11), direkt beschichtet mit einer Schicht aus transparenter Beschichtung (112), wobei die Beschichtung (112) aus einer Mischung aus einem Bindemittel und mindestens einem Pigment hergestellt ist, wobei das Bindemittel ausgewählt ist aus der Gruppe, bestehend aus Polyvinylalkohol, Polyacrylat, Polyvinylacetat und Styrol/Butadien-Kautschuk, wobei das Pigment ausgewählt ist aus der Gruppe, bestehend aus Titandioxid, Calciumcarbonat, Tonerde und Mischung derselben, wobei das Gewichtsverhältnis von Bindemittel zu Pigment von 1 : 1 bis 1 : 10 reicht.

2. Schreibbogen nach Anspruch 1, **dadurch gekennzeichnet, dass** der Kunststofffilm (11) hergestellt ist aus einem Material, ausgewählt aus der Gruppe, bestehend aus Polypropylen, Polyethylen, Polyvinylchlorid und Polyethylenterephthalat.

3. Schreibbogen nach Anspruch 1 oder Anspruch 2, zusätzlich **gekennzeichnet durch** eine Schicht aus einem entfernbaren Adhesiv (111), aufgetragen auf den Kunststofffilm (11), um den Schreibbogen (1) mit einer entfernbar haftenden Eigenschaft zu versehen.

4. Schreibbogen nach einem der Ansprüche 1 bis 3, zusätzlich **gekennzeichnet durch** ein Trennpapier, dass die Beschichtung (112) des Kunststofffilms (11) bedeckt.

5. Schreibbogen nach Anspruch 1, **dadurch gekennzeichnet, dass** das Bindemittel Polyvinylalkohol und das Pigment Titandioxid ist, worin das Gewichtsverhältnis von Polyvinylalkohol zu Titandioxid von 1 : 1 bis 1 : 2 beträgt.

6. Schreibbogen nach Anspruch 1, **dadurch gekennzeichnet, dass** das Bindemittel Styrol/Butadien-Kautschuk und das Pigment Calciumcarbonat ist, worin das Gewichtsverhältnis von Styrol/Butadien-Kautschuk zu Calciumcarbonat von 1 : 1 bis 1 : 2 beträgt.

7. Schreibbogen nach Anspruch 1, **dadurch gekennzeichnet, dass** die Beschichtung zusätzlich einen Farbstoff enthält.

## Revendications

1. Feuille pour l'écriture **caractérisée par** un film en plastique transparent (11) revêtu directement avec une couche de revêtement transparent (112), ladite couche de revêtement (112) étant préparée à partir d'un mélange d'un liant et d'au moins un pigment, ledit liant étant choisi parmi le groupe constitué par l'alcool polyvinylique, le polyacrylate, l'acétate de polyvinyle et le caoutchouc styrène-butadiène, ledit pigment étant choisi parmi le groupe constitué par le dioxyde de titane, le carbonate de calcium, l'argile et leurs mélanges, le rapport pondéral dudit liant audit pigment se situant de 1 : 1 à 1 : 10.

2. Feuille pour l'écriture selon la revendication 1, **caractérisée en ce que** ledit film en plastique (11) est constitué d'un matériau choisi parmi le groupe constitué par le polypropylène, le polyéthylène, le chlorure de polyvinyle et le téréphtalate de polyéthylène.

3. Feuille pour l'écriture selon la revendication 1 ou la revendication 2, **caractérisée, en outre, par** une couche d'adhésif amovible (111) appliquée audit film en plastique (11) pour munir ladite feuille pour l'écriture (1) d'une caractéristique d'adhésivité amovible.

4. Feuille pour l'écriture selon l'une quelconque des revendications 1 à 3, **caractérisée, en outre, par** un intercalaire qui recouvre ladite couche de revêtement (112) dudit film plastique (11).

5. Feuille pour l'écriture selon la revendication 1, **caractérisée en ce que** ledit liant est de l'alcool polyvinylique et ledit pigment est du dioxyde de titane, dans laquelle le rapport pondéral de l'alcool polyvinylique au dioxyde de titane est de 1 : 1 à 1 : 2.

6. Feuille pour l'écriture selon la revendication 1, **caractérisée en ce que** ledit liant est du caoutchouc styrène-butadiène et ledit pigment est du carbonate de calcium, dans laquelle le rapport pondéral du caoutchouc styrène-butadiène au carbonate de calcium est de 1 : 1 à 1 : 2.

7. Feuille pour l'écriture selon la revendication 1, **caractérisée en ce que** ledit revêtement comprend, en outre, un colorant.
